# EUROPEAN PATENT SPECIFICATION

(11) **EP 1 042 765 B1**
(45) Date of publication and mention of the grant of the patent: **09.05.2007**
(21) Application number: 98962060.4
(22) Date of filing: 10.12.1998
(51) Int. Cl.: H01C 7/02, H01C 17/30

(54) **METHOD OF MAKING AN ELECTRICAL DEVICE**
VERFAHREN ZUR HERSTELLUNG EINER ELEKTRISCHEN VORRICHTUNG
METHODE DE FABRICATION D'UN DISPOSITIF ELECTRIQUE

(30) Priority: 15.12.1997 US 990707
(43) Date of publication of application: 11.10.2000
(73) Proprietor: TYCO Electronics Corporation, Menlo Park, CA 94025-1164 (US)
(72) Inventor: MIYASAKA, Naofumi, Narita, Chiba (JP); FANG, Shou-mean, 2419 Hong Qiao Road, Shanghai 200335 (CN)
(74) Representative: Jay, Anthony William
(86) International application number: PCT/US1998/026328
(87) International publication number: WO 1999/031677

(56) References cited:
- EP-A- 0 344 734
- EP-A- 0 484 138
- EP-A- 0 522 863
- EP-A- 0 730 282
- EP-A- 0 844 622

## Description

### Field of the Invention

This invention relates to a method of making electrical devices comprising conductive polymers, and a method of making a battery assembly.

### Introduction to the Invention

Electrical devices which comprise conductive polymer compositions which exhibit PTC (positive temperature coefficient of resistance) behavior are well-known and are used as circuit protection devices and heaters. Such circuit protection devices, containing low resistivity conductive polymer compositions, respond to changes in ambient temperature and/or current conditions. Under normal conditions, a circuit protection device remains in a low temperature, low resistance state when in series with a load in an electrical circuit When exposed to an overcurrent or overtemperature condition, however, the device increases in resistance, effectively shutting down the current flow to the load in the circuit. For many applications it is desirable that the device have as low a resistance as possible in order to minimize the contribution to the total resistance of the electrical circuit during normal operation. Furthermore, a low resistance allows the device to have a higher hold current, i.e. the largest steady state current that, under specified ambient conditions, can be passed through a circuit protection device without causing the device to "trip" into the high resistance state. Although low resistance devices can be made from a given composition by changing dimensions, e.g. making the distance between the electrodes very small or the device area very large, small devices are preferred. Such devices occupy less space on a circuit board and generally have desirable thermal properties.

EP-A- 0730282 discloses a PTC element comprising a conductive sheet of a crystalline polyolefin matrix, and a conductive filler, having provided on both sides thereof an electrode of a metallic foil.

### BRIEF SUMMARY OF THE INVENTION

The most common technique to achieve a small device is to use a composition that has a low resistivity. It is known that various processing steps, e.g. irradiation, encapsulation, or exposure to elevated temperature during solder reflow, can increase the resistivity of the composition during device fabrication. Therefore, it is desirable to use processing techniques which increase the resistivity of the composition as little as possible so that the final device will have a low resistance. We have now found a particular sequence of processing steps which helps in producing a device with a low resistance. In a first aspect this invention provides a method of making an electrical device which comprises
(A) a resistive element which is composed of a conductive polymer composition which exhibits PTC behavior and which comprises
   (1) a polymeric component having a crystallinity of at least 20% and a melting point Tm, and
   (2) dispersed in the polymeric component, a particulate conductive filler; and
(B) two electrodes which (i) are attached to the resistive element, (ii) comprise metal foils, and (iii) can be connected to a source of electrical power,
the method comprising the steps of
(a) cutting a device from a laminate comprising the conductive polymer composition positioned between two metal foils;
(b) exposing the device after the cutting step to at least one thermal excursion from a first temperature which is at most (Tₘ - 100)°C to a second temperature which is at most (Tₘ - 25)°C; and
   **characterised in that** the method further comprises
(c) crosslinking the conductive polymer composition after the thermal excursion.

The invention also provides a method for making a battery assembly which comprises the steps of
(1) providing a battery which comprises first and second terminals; and
(2) producing a device according to the first aspect of the invention which further comprises (a) attaching a first conductive lead to the first electrode of said device, and (b) attaching a second conductive lead to the second electrode of said device;
(3) placing said device in contact with the first terminal of the battery so that the first conductive lead is in physical and electrical contact with that terminal.

### BRIEF DESCRIPTION OF THE DRAWINGS

The invention is illustrated by the drawings in which Figure 1 is a cross-sectional view of a device produced by the method of the invention;
Figure 2 is a top view of a device produced by the method of the invention;
Figure 3 is a top view of a first conductive lead which forms part of a device produced by the method of the invention ;
Figure 4 is a top view of a device produced by the method of the invention with a second conductive lead attached;
Figure 5 is a top view of a device produced by the method of the invention comprising an insulating layer; and
Figure 6 is a graph showing the resistance distribution for devices made by a method of the invention and two comparative methods.

### DETAILED DESCRIPTION OF THE INVENTION

The electrical device produced by the method of the invention comprises a resistive element composed of a conductive polymer composition, and first and second metal foil electrodes which are attached to, and sandwich, the resistive element The conductive polymer composition comprises a polymeric component, and dispersed therein, a particulate conductive filler. The polymeric component comprises one or more polymers, one of which is preferably a crystalline polymer having a crystallinity of at least 20% as measured in its unfilled state by a differential scanning calorimeter. Suitable crystalline polymers include polymers of one or more olefins, particularly polyethylene such as high density polyethylene; copolymers of at least one olefin and at least one monomer copolymerisable therewith such as ethylene/acrylic acid, ethylene/ethyl acrylate, ethylene/vinyl acetate, and ethylene/butyl acrylate copolymers; melt-shapcable fluoropolymers such as polyvinylidene fluoride (PVDF) and ethylene/tetrafluoroethylene copolymers (ETFE, including terpolymers); and blends of two or more such polymers. For some applications it may be desirable to blend one crystalline polymer with another polymer, e.g. an elastomer or an amorphous thermoplastic polymer, in order to achieve specific physical or thermal properties, e.g. flexibility or maximum exposure temperature. The polymeric component generally comprises 40 to 90% by volume, preferably 45 to 80% by volume, especially 50 to 75% by volume of the total volume of the composition.

The particulate conductive filler which is dispersed in the polymeric component may be any suitable material, including carbon black, graphite, metal, metal oxide, conductive coated glass or ceramic beads, particulate conductive polymer, or a combination of these. The filler may be in the form of powder, beads, flakes, fibers, or any other suitable shape. The quantity of conductive filler needed is based on the required resistivity of the composition and the resistivity of the conductive filler itself. For many compositions the conductive filler comprises 10 to 60% by volume, preferably 20 to 55% by volume, and for low resistivity compositions used for low resistance circuit protection devices, especially 25 to 50% by volume of the total volume of the composition.

The conductive polymer composition may comprise additional components, such as antioxidants, inert fillers, nonconductive fillers, radiation crosslinking agents (often referred to as prorads or crosslinking enhancers, e.g. triallyl isocyanurate), stabilizers, dispersing agents, coupling agents, acid scavengers (e.g. CaCO₃), or other components. These components generally comprise at most 20% by volume of the total composition. Dispersion of the conductive filler and other components into the polymeric component may be achieved by any suitable means of mixing, e.g. melt-processing or solvent-mixing. The mixed composition can be melt-shaped by any suitable method, e.g. melt-extrusion, injection-molding, compression-molding, or sintering, in order to produce a resistive element. The element is preferably laminar and may be of any shape, e.g. rectangular, square, circular, or annular. The resistive element often has a thickness of at most 1.02 mm (0.040 inch), and, for many applications, is much thinner, i.e. has a thickness of at most 0.51 mm (0.020 inch), preferably at most 0.38 mm (0.015 inch).

The composition used in the resistive element exhibits positive temperature coefficient (PTC) behavior, i.e. it shows a sharp increase in resistivity with temperature over a relatively small temperature range. In this application, the term "PTC" is used to mean a composition or device which has an R₁₄ value of at least 2.5 and/or an R₁₀₀ value of at least 10, and it is preferred that the composition or device should have an R₃₀ value of at least 6, where R₁₄ is the ratio of the resistivities at the end and the beginning of a 14°C range, R₁₀₀ is the ratio of the resistivities at the end and the beginning of a 100°C range, and R₃₀ is the ratio of the resistivities at the end and the beginning of a 30°C range. Generally the compositions used in devices of the invention show increases in resistivity which are much greater than those minimum values.

Suitable conductive polymer compositions are disclosed in U.S. Patent Nos. 4,237,441 (van Konynenburg et al), 4,545,926 (Fouts et al), 4,724,417 (Au et al), 4,774,024 (Deep et al), 4,935,156 (van Konynenburg et al), 5,049,850 (Evans et al), 5,250,228 (Baigrie et al), 5,378,407 (Chandler et al), 5,451,919 (Chu et al), 5,582,770 (Chu et al), 5,747,147 (Wartenberg et al), and 5,801,612 (Chandler et al), and in commonly assigned International Publication No. WO96/29711 (Raychem Corporation, published September 26, 1997).

The resistive element is attached to first and second laminar electrodes which are attached to the first face and the second face, respectively, of the resistive element. It is preferred that the conductive polymer composition be extruded or otherwise formed into a sheet onto which the electrodes may be attached to form a laminate, i.e. the conductive polymer is sandwiched between the foils. Both first and second electrodes comprise a conductive material, and are preferably metal in the form of a foil, e.g. nickel, copper, brass, stainless steel, or an alloy of one or more of these metals, although one or both of the electrodes may comprise a conductive paint or graphite layer. A tie layer, e.g. a conductive adhesive, may be used to attach the electrode to the resistive element. It is particularly preferred that the first and second electrodes comprise an electrodeposited metal foil, e.g. nickel, copper, or nickel-coated copper. Appropriate electrodes are disclosed in U.S. Patents Nos. 4,689,475 (Matthiesen) and 4,800,253 (Kleiner et al), and in International Publication No. WO95/34081 (Raychem Corporation, published December 14, 1995).

The device may also comprise an insulating layer, which provides electrical and environmental protection to the device. The insulating layer generally covers some or all of the metal foil electrodes and any exposed surfaces of the resistive element. Suitable insulating materials include polymers such as polyamide, polybutylene terephthalate, a polyester, polyethylene, polyvinylidene fluoride, liquid crystalline polymers, or an epoxy resin.

In the method of the invention, in a cutting step, the device is cut from a laminate comprising the conductive polymer composition positioned between two metal foils. In this application, the term "cutting" is used to include any method of isolating or separating the resistive element of the device from the laminate, e.g. dicing, punching, shearing, cutting, etching and/or breaking as described in International Publication No. WO95/34084 (published December 14, 1995).

The device is then subjected to a thermal treatment step. The thermal treatment step comprises at least one excursion from a first temperature T₁ to a second temperature T₂. Preferably the thermal treatment step includes a return to the first temperature after exposure to the second temperature, thus creating a cycle from T₁ to T₂ to T₁. The first temperature is at most (Tₘ - 100)°C, preferably at most (Tₘ - 120)°C, particularly at most (Tₘ - 150)°C, where Tₘ is the melting point of the polymeric component, as measured by the peak of the endotherm of a differential scanning calorimeter. When there is more than one peak, for example when the polymeric component comprises a mixture of crystalline polymers, Tₘ, is defined as the temperature of the highest temperature peak. The second temperature is at most (Tₘ - 25)°C, preferably at most (Tₘ - 35)°C, particularly at most (Tₘ - 50)°C. It is important that the first temperature be at a temperature above the glass transition temperature T_{g} of the polymeric component. T₁ is often at a temperature below room temperature, i.e. less than 20°C. In a preferred embodiment of the method, the device is exposed to at least two thermal cycles, preferably at least three thermal cycles. For some applications, the device may be exposed to many more thermal cycles, e.g. six thermal cycles. During the thermal treatment step, for the thermal excursion or for each thermal cycle, the device is held at both the first and the second temperatures for sufficient time to ensure that the entire device reaches the designated temperature. The time period during which the device is held may be the same or different at T₁ and T₂, but is generally at least 1 minute, preferably at least 3 minutes, more preferably at least 5 minutes, particularly at least 10 minutes, more particularly at least 15 minutes, especially at least 30 minutes, e.g. 60 minutes, as measured from the time the device reaches the designated temperature. Any suitable heat source may be used during the thermal treatment step, e.g. an oven (particularly a programmable oven) or other environmental chamber, or a heat lamp. The rate of temperature increase from T₁ to T₂ (and back to T₁, if present), may be any convenient rate, e.g. 2 to 30°C/minute. When the thermal treatment step is a thermal cycle, the rate from T₁ to T₂ may the same as or different from the rate from T₂ to T₁.

Following the thermal treatment step, the conductive polymer composition is crosslinked. Crosslinking can be accomplished by chemical means or by irradiation, e.g. using an electron beam or a Co⁶⁰ γ irradiation source. The level of crosslinking depends on the required application for the composition, but is generally less than the equivalent of 200 Mrads, and is preferably substantially less, i.e. from 1 to 20 Mrads, preferably from 1 to 15 Mrads, particularly from 2 to 10 Mrads for low voltage (i.e. less than 60 volts) applications. Useful circuit protection devices for applications of less than 30 volts can be made by irradiating the device to at least 2 Mrads but at most 10 Mrads.

For many applications, it is necessary to attach at least one conductive lead, i.e. a first conductive lead, to one of the metal foil electrodes. Often first and second conductive leads are attached to first and second electrodes, respectively. The conductive leads allow easy connection of the electrodes to the source of electrical power, e.g. a battery or a power source, or into the circuit, and can be used to control the thermal output of the device. The conductive leads, which often are supplied as part of a lead frame for ease in manufacture, are preferably attached to the electrodes by means of an intermediate layer, e.g. solder or a conductive adhesive. This lead attachment step preferably occurs after the cutting step and before the thermal treatment step. Other assembly processes, e.g. application of the electrically insulating layer such as an epoxy resin or other polymer, are preferably conducted during an assembly step, which includes the lead attachment step and occurs after the cutting step and before the thermal treatment step.

Following the method of the invention, devices in which the conductive polymer has a low resistivity, i.e. less than 100 ohm-cm, preferably less than 20 ohm-cm, particularly less than 10 ohm-cm, more particularly less than 5 ohm-cm, especially less than 2 ohm-cm, e.g. less than 1 ohm-cm, can be prepared. For most applications, the device generally has a resistance at 20°C of less than 1 ohm, preferably less than 0.5 ohms, particularly less than 0.25 ohms, e.g. 0.050 to 0.150 ohms.

Devices made by the method according to the invention are particularly suitable for use in a battery assembly, in which the device is preferably attached to the first or second terminal of a battery. The attachment may be directly between the battery and the first or second electrode, or between the battery and the first conductive lead which is attached to the first electrode, or the second conductive lead which is attached to the second electrode. For some batteries, in which either the first and/or the second terminal is in the form of a "button", the device is physically and electrically attached to a button terminal. The device may be attached to either the negative or the positive terminal of the battery. Batteries suitable for use include nickel-cadmium, nickel-metal hydride, alkaline, or lithium batteries. Often the battery assembly comprises two or more batteries. Such a battery assembly is shown in International Publications Nos. WO97/06538 (K.K. Raychem, published February 20, 1997) and WO98/20567 (Raychem Corporation, published May 14, 1998).

The invention is illustrated by the drawings in which Figure 1 shows in cross-section electrical device 1 comprising PTC component 3, first conductive lead 15, second conductive lead 18, and insulating material 23. PTC component 3 comprises first electrode 11, second electrode 13 and resistive element 9 composed of a conductive polymer sandwiched therebetween. In PTC component 3 shown in Figure 1, both electrodes opposing each other form first surface 43 and second surface 41.

A top view of PTC component 3 is shown in Figure 2. PTC component 3 comprises surfaces 41 and 43, outer periphery 5 and inner periphery 7 and is in the form of a disk with an opening 27 in the center. The inner periphery 7 defines the opening 27.

Figure 3 shows a top view of first conductive lead 15, which has a first part 16 which is attached to first electrode 11, and a second part 17 which extends across opening 27 of PTC component 3. In this embodiment, first part 16 covers the whole surface of first electrode 11. Second part 17 of first lead 15, which covers at least a part of opening 27, is used to make direct electrical contact, via solder, pressure, or a weld, to a button terminal of a battery. The second part 17 covers at least a part of opening 27.

Figure 4 shows a top view of second conductive lead 18, which comprises first part 19 and second part 21. First part 19 is attached to second electrode 13 and covers at least part of the surface of second electrode 13. Second part 21 extends away from outer periphery 5 and can be bent, if necessary, to make electrical contact to a second battery or other electrical component. First and second conductive leads 15,18 can be made from any suitable material, e.g. nickel, stainless steel, copper, or an alloy such as brass or bronze. For ease of manufacture second lead 18 is often part of a lead frame.

Figure 5 shows a top view of device 1 which as been encapsulated by electrically insulating layer 23. When a positive terminal of a battery is placed inside opening 27', no short circuit occurs because no electrical contact is made between the terminal and PTC component 3.

The invention is illustrated by the following examples, in which Examples 1 and 2 are comparative examples. The following steps were conducted for each example:

### Preparation of PTC Device

A first compound was prepared by preblending 54% by weight carbon black (Raven^{™} 430U, available from Columbian Chemicals) with 46% by weight high density polyethylene (Petrothene^{™} LB832, available from Millenium; "HDPE") in a Henschel blender, mixing the blend in a Buss kneader, and extruding into pellets. A second compound was prepared by preblending 51.4% by weight carbon black with 48.6% by weight HDPE in the same way. Pellets of the first and second compounds were preblended to give a final compound having 52.7% by weight carbon black and 47.3% by weight HDPE, and this compound was extruded through a sheet die using an Egan extruder to give a sheet with a thickness of 0.25 mm (0.010 inch). The extruded sheet was laminated between two layers of electrodeposited nickel foil having a thickness of about 0.033 mm (0.0013 inch) (available from Fukuda) by using a press set at 200°C. The laminated sheet was solder-dipped into a solder formulation of 63% lead/37% tin heated to 230°C, and devices having the shape shown in Figure 2 were punched from the laminated sheet.

### Assembly of Device

First and second conductive leads, as shown in Figures 3 and 4, were attached to the PTC device by means of 63/37 lead/tin solder, which was reflowed in a hot-air oven which increased in temperature from 30°C to a maximum temperature of 230°C over about 2 minutes. An insulating layer of liquid crystalline polymer was then applied by means of transfer or injection molding.

### Irradiation

Devices were irradiated by using a cobalt 60 γ irradiation source to give a total irradiation of 14 Mrad.

### Temperature Cycling

The devices were thermally cycled six times, each cycle being from -40 to 80 to - 40°C at a rate of 1°C/minute with a 60 minute dwell at -40°C and 80°C.

### Examples 1 and 2 (Comparative)

Device preparation was conducted as shown in Table I, with numbers 1 to 4 indicating the sequential order of the process steps as they were conducted. The resistance at 25°C was measured for one hundred devices prepared for each example. The resulting devices had an average resistance at least 5% higher than that of devices of the invention (Example 3).

### Example 3

Device preparation was conducted as shown in Table I. The resulting devices had a resistance lower than that of conventional devices. A comparison of the resistance distribution of the devices is shown in Figure 6.

| Example | Device Preparation Steps | | | | Resistance (mohms) |
|---|---|---|---|---|---|
| | Preparation | Assembly | Irradiation | Temp.Cycle | |
| 1 | 1 | 2 | 3 | 4 | 53.3 |
| 2 | 1 | 3 | 2 | 4 | 64.9 |
| 3 | 1 | 2 | 4 | 3 | 49.0 |

## Claims

1. A method of making an electrical device (1) which comprises
(A) a resistive element (9) which is composed of a conductive polymer composition which exhibits PTC behavior and which comprises
(1) a polymeric component having a crystallinity of at least 20% and a melting point Tₘ, and
(2) dispersed in the polymeric component, a particulate conductive filler; and
(B) two electrodes (11,13) which (i) are attached to the resistive element (9), (ii) comprise metal foils, and (iii) can be connected to a source of electrical power,
the method comprising the steps of
(a) cutting a device (1) from a laminate comprising the conductive polymer composition positioned between two metal foils;
(b) exposing the device (1) after the cutting step to at least one thermal excursion from a first temperature which is at most (Tₘ - 100)°C to a second temperature which is at most (Tₘ - 25)°C; and
**characterised in that** the method further comprises
(c) crosslinking the conductive polymer composition after the thermal excursion.

2. A method according to claim 1 which comprises attaching at least one conductive lead (15) to one of the metal foil electrodes after step (a) and before step (b).

3. A method according to claim 1 or 2, which the device (1) has been crosslinked in step (c) to the equivalent of 1 to 20 Mrads.

4. A method according to any one of the preceding claims wherein the polymeric component comprises polyethylene, an ethylene copolymer, or a fluoropolymer.

5. A method according to any one of the preceding claims wherein in step (b) the device (1) is exposed to at least one thermal cycle from the first temperature to the second temperature and back to the first temperature.

6. A method according to any one of the preceding claims wherein in step (b) the first temperature T₁ is less than 23°C.

7. A method according to claim 1 wherein
(1) the resistive element (9) (i) has a thickness of at most O.S mm and (ii) is crosslinked to the equivalent of at least 2 Mrads, and
(2) in step (b), the device (1) is exposed to at least one thermal cycle from a first temperature which is at most (Tₘ - 100)°C to a second temperature which is at most (Tₘ- 25)°C and back to the first temperature after the cutting step.

8. A method according to claim 7 wherein in step (b) the device (1) is exposed to at least three thermal cycles.

9. A method for making a battery assembly comprising the steps of
(1) providing a battery which comprises first and second terminals; and
(2) producing a device (1) according to claim 1 (a) and attaching a first conductive lead (15) to the first electrode (11) of said device (1) and (b) attaching a second conductive lead (18) to the second electrode (13) of said device (1);
(3) placing (1) said device in contact with the first terminal of the battery so that the first conductive lead (15) is in physical and electrical contact with that terminal.

## Patentansprüche

1. Verfahren zur Herstellung einer elektrischen Vorrichtung (1), die folgendes umfaßt:
(A) ein Widerstandselement (9), das aus einer leitfähigen Polymerzusammensetzung zusammengesetzt ist, die PTC-Verhalten zeigt und die folgendes umfaßt:
(1) eine Polymerkomponente mit einer Kristallinität von mindestens 20% und einem Schmelzpunkt Tₘ und
(2) einen in der Polymerkomponente dispergierten partikelförmigen leitfähigen Füllstoff; und
(B) zwei Elektroden (11, 13), die (i) an dem Widerstandselement (9) befestigt sind, (ii) Metallfolien umfassen und (iii) mit einer elektrischen Stromquelle verbunden werden können,
wobei das Verfahren die folgenden Schritte umfaßt:
(a) Abschneiden einer Vorrichtung (1) von einem Schichtwerkstoff, der die zwischen zwei Metallfolien positionierte leitfähige Polymerzusammensetzung umfaßt;
(b) Aussetzen der Vorrichtung (1) nach dem Abschneideschritt mindestens einer Temperaturexkursion von einer ersten Temperatur, die höchstens (Tₘ - 100)°C beträgt, bis zu einer zweiten Temperatur, die höchstens (Tₘ - 25)°C beträgt; und
**dadurch gekennzeichnet, daß** das Verfahren ferner den folgenden Schritt umfaßt:
(c) Vernetzen der leitfähigen Polymerzusammensetzung nach der Temperaturexkursion.

2. Verfahren nach Anspruch 1, das den folgenden Schritt umfaßt: Befestigen mindestens eines leitfähigen Leiters (15) an einer der Metallfolien-Elektroden nach Schritt (a) und vor Schritt (b).

3. Verfahren nach Anspruch 1 oder 2, bei dem die Vorrichtung (1) in Schritt (c) zu dem Äquivalent von 1 bis 20 Mrads vernetzt worden ist.

4. Verfahren nach einem der vorhergehenden Ansprüche, wobei die Polymerkomponente Polyethylen, ein Ethylen-Copolymer oder ein Fluorpolymer umfaßt.

5. Verfahren nach einem der vorhergehenden Ansprüche, wobei die Vorrichtung (1) in Schritt (b) mindestens einem thermischen Zyklus von der ersten Temperatur zur zweiten Temperatur und zurück zur ersten Temperatur ausgesetzt wird.

6. Verfahren nach einem der vorhergehenden Ansprüche, wobei in Schritt (b) die erste Temperatur T₁ weniger als 23 °C beträgt.

7. Verfahren nach Anspruch 1, wobei:
(1) das Widerstandselement (9) (i) eine Dicke von höchstens 0,51 mm hat und (ii) zu dem Äquivalent von mindestens 2 Mrads vernetzt wird und
(2) in Schritt (b) die Vorrichtung (1) nach dem Abschneideschritt mindestens einem thermischen Zyklus von einer ersten Temperatur, die höchstens (Tₘ - 100)°C beträgt, bis zu einer zweiten Temperatur, die höchstens (Tₘ - 25)°C beträgt, und zurück zur ersten Temperatur ausgesetzt wird.

8. Verfahren nach Anspruch 7, wobei die Vorrichtung (1) in Schritt (b) mindestens drei thermischen Zyklen ausgesetzt wird.

9. Verfahren zur Herstellung einer Batterieanordnung, die folgenden Schritte umfassend:
(1) Bereitstellen einer Batterie, die einen ersten und einen zweiten Anschluß umfaßt; und
(2) Herstellen einer Vorrichtung (1) nach Anspruch 1und
(a) Befestigen einer ersten leitfähigen Leitung (15) an der ersten Elektrode (11) der Vorrichtung (1) und
(b) Befestigen eines zweiten leitfähigen Leitung (18) an der zweiten Elektrode (13) der Vorrichtung (1);
(3) Inkontaktbringen der Vorrichtung (1) mit dem ersten Anschluß der Batterie, so daß die erste leitfähige Leitung (15) in physischem und elektrischem Kontakt mit diesem Anschluß ist.

## Revendications

1. Méthode pour fabriquer un dispositif électrique (1) qui comprend
(A) un élément résistif (9) qui est composé d'une composition de polymère conducteur qui présente un comportement CTP et qui comprend
(1) un composant polymérique ayant une cristallinité d'au moins 20% et un point de fusion Tₘ, et
(2) dispersé dans le composant polymérique, un bourrage conducteur particulaire; et
(B) deux électrodes (11, 13) qui (i) sont attachées à l'élément résistif (9), (ii) comprennent des feuilles de métal, et (iii) peuvent être connectées à une source d'énergie électrique,
la méthode comprenant les étapes
(a) de découper un dispositif (1) à partir d'un laminé comprenant la composition de polymère conducteur positionnée entre deux feuilles de métal;
(b) d'exposer le dispositif (1) après l'étape de découpage à au moins un passage thermique allant d'une première température qui est au plus (Tₘ - 100)°C à une seconde température qui est au plus (Tₘ - 25)°C; et
**caractérisée en ce que** la méthode comprend en outre
(c) réticuler la composition de polymère conducteur après l'augmentation thermique.

2. Méthode selon la revendication 1, qui comprend l'attachement d'au moins un fil conducteur (15) à une des électrodes en feuille de métal après l'étape (a) et avant l'étape (b).

3. Méthode selon la revendication 1 ou 2, dans laquelle le dispositif (1) a été réticulé à l'étape (c) à l'équivalent de 1 à 20 Mrads.

4. Méthode selon l'une quelconque des revendications précédentes, dans laquelle le composant polymérique comprend du polyéthylène, un copolymère d'éthylène, ou un fluoropolymère.

5. Méthode selon l'une quelconque des revendications précédentes, dans laquelle à l'étape (b) le dispositif (1) est exposé à au moins un cycle thermique allant de la première température à la seconde température et revenant à la première température.

6. Méthode selon l'une quelconque des revendications précédentes, dans laquelle à l'étape (b) la première température T₁ est inférieure à 23°C.

7. Méthode selon la revendication 1, dans laquelle
(1) l'élément résistif (9) (i) a une épaisseur d'au plus 0,51 mm et (ii) est réticulé à l'équivalent d'au moins 2 Mrads, et
(2) à l'étape (b), le dispositif (1) est exposé à au moins un cycle thermique allant d'une première température qui est au plus (Tₘ - 100)°C à une seconde température qui est au plus (Tₘ - 25)°C et revenant à la première température après l'étape de découpage.

8. Méthode selon la revendication 7, dans laquelle à l'étape (b) le dispositif (1) est exposé à au moins trois cycles thermiques.

9. Méthode pour fabriquer un assemblage de batterie comprenant les étapes; et
(1) de fournir une batterie qui comprend des premières et secondes bornes; et
(2) de produire un dispositif (1) selon la revendication 1 et
(a) attacher un premier fil conducteur (15) à la première électrode (11) dudit dispositif (1), et
(b) attacher un second fil conducteur (18) à la seconde électrode (13) dudit dispositif (1);
(3) de placer ledit dispositif (1) en contact avec la première borne de la batterie de telle sorte que le premier fil conducteur (15) est en contact physique et électrique avec cette borne.
